

Feb. 11, 1941.

E. O. NORRIS

2,231,678

MATRIX FOR ELECTROFORMING FORAMINOUS SHEETS

Filed April 21, 1938



INVENTOR  
EDWARD O. NORRIS

BY  
John H. Billiard  
ATTORNEY

## UNITED STATES PATENT OFFICE

2,231,678

MATRIX FOR ELECTROFORMING  
FORAMINOUS SHEETS

Edward O. Norris, Westport, Conn., assignor to  
Edward O. Norris, Inc., New York, N. Y., a corporation of New York

Application April 21, 1938, Serial No. 203,235

7 Claims. (Cl. 204—11)

My present invention relates to matrices, and more particularly to an improved matrix and the method of making the same.

In my issued Patents 2,166,366 and 2,166,367, both issued July 18, 1939, I have described and claimed the improved method of making a matrix on which may be electro-deposited a suitable metal, such as copper, to form a foraminous plate or sheet. My present invention, as regards the method of making a matrix, and the resulting matrix, while somewhat analogous to those of my co-pending applications referred to, is an improvement thereover.

According to my present invention, as in the inventions described and claimed in my co-pending applications referred to, I produce a matrix having a face of electrically conductive material arranged in the form of any desired pattern and with the material between the lands of the pattern comprising material that presents a surface inactive to electrolytic deposition, such as fillings of commercial Bakelite, or other similar phenolic condensation product, asphaltum, natural and synthetic rubber, or a thick plating of chromium (say .001") on metal. Such material I will term hereinafter "passive material."

As a part of my invention, I describe an improved means of locking the passive material to the matrix and thus produce a matrix on which foraminous sheets or plates may be electro-deposited and then stripped therefrom without injury to the matrix.

Generally described, the object of the invention is an improved matrix adapted for producing by electro-deposition foraminous sheet material and having the characteristics of durability, so that repeated deposits may be made thereon and stripped therefrom, and also cheapness of production and resistance to disintegration by corrosion.

Another object consists in a method of producing such a matrix.

In the accompanying drawing:

Fig. 1 is a section through a portion of a matrix and illustrating the first step of my improved method;

Fig. 2 is a section through a portion of a matrix and illustrating another step of my improved method;

Fig. 3 is a section through a portion of a matrix and illustrating a further step of my improved method;

Fig. 4 is a section through a portion of a complete matrix made according to my improved method;

Fig. 5 is a perspective view of a complete matrix

partly in section, made according to my improved method.

In producing a matrix according to my present invention, a metallic plate or matrix base 10 composed, for example, of copper and produced in any desired manner, such as by the photo-printing and etching method described in my Patent No. 2,166,366, is provided on one face for instance with a plurality of lands 11 arranged, if a square mesh foraminous sheet is to be made, at 10 right angles to each other so as to exhibit a surface having the pattern of a network of interconnected lands separated by depressions or pits 12. While the lands are preferably arranged at right angles to each other, I may arrange them 15 at any other desired angle and the showing therefore is to be considered as merely illustrative. Proceeding with the plate thus described, the pitted face thereof is treated by coating it with shellac 13 so that the surfaces of the pits 20 and the lands are entirely covered. The surface of the plate is then treated by rubbing or grinding, or a like method, until the shellac is completely removed from the surfaces of the lands. The next step consists in covering the entire surface of the plate, including the shellac-covered surfaces of the pits and the exposed metallic surface of the lands, with conducting material 14 to which an electrolytic deposit thereon does not 25 adhere with enough tenacity to prevent it from 30 being readily stripped off. An example of a suitable substance for the purpose is a mixture of wax and graphite having about the consistency of thin paste. This paste is applied to the face of the plate 10, entirely covering the lands and 35 the surfaces of the pits, and thus serving as a depositing surface to which, however, the deposit does not tenaciously adhere. As an alternative to this procedure, the wax may first be applied, and, after it is thoroughly rubbed out thin, the 40 graphite or bronze powder or some other electrically conductive powder may be dusted over the surface.

The next step is to employ the plate thus prepared as a cathode in an electrolytic bath and 45 deposit thereon the layer 15—say of copper, building up the deposit to a substantial thickness in the order, for example, of .005" or .010". Those parts of the plate which are to be excluded from the electrolytic action may be masked in any of 50 the several ways known in the art.

The deposit 15 may then be stripped from the plate 10 and employed as the foundation plate of an intermediate matrix to be used for the production of the final matrix.

Referring to Fig. 2, the base plate is shown with an asphaltum mask 18 to protect it against electrolytic action and with the depressions 17 filled with shellac 16 and additional deposits 19 which flow over the edges of the shellac fillings 16. The shellac filling is applied by covering the entire surface of the base plate with shellac and then rubbing off the protuberances 18a. The additional deposits 19 are produced by subjecting the base plate with its shellac fillings and asphaltum backing to electrolytic deposition until the deposit on the exposed areas has reached a substantial thickness.

To produce the final matrix, the shellac 16 is washed out with alcohol or other suitable solvent and the plate is then employed as a depositing surface on which to electroform the layer 21. If the plate 15 and the built-up portions 19 are of copper, the deposit 21 should be of material that is not affected by a re-agent that corrodes copper or, more generally speaking, the plate 15 with its built-up portions 19 must be capable of removal from the deposit 21 by some agency, presently to be referred to, that acts selectively on it to the exclusion of action on the nickel. It is to be noted that the process carried to the point shown in Fig. 2 has resulted in protuberances 19 that are peripherally grooved as shown at 20. Therefore, the nickel deposit 21 conforms to the surface contour of these grooves as well as to the surface contour of the remaining areas of the plate 15, resulting in depressions, about each wall of which there is an inwardly extending overhanging ledge or shoulder 25.

After removing the asphaltum mask 18, the copper plate 15 and its protuberances 19 may be removed by electrolytic deplating in a bath such that the nickel is not affected, or by the application of (1) a solution of potassium cyanide, or (2) a mixture of chromic and sulphuric acids in water, suitable proportions being about as follows:

|                |              |    |
|----------------|--------------|----|
| Sulphuric acid | -----pounds  | 2  |
| Chromic acid   | -----pound   | 1  |
| Water          | -----gallons | 10 |

Either of these agents acts on the copper to the exclusion of the nickel.

The entire metallic surface of the nickel deposit now being exposed, the nickel deposit may be strengthened by the deposit 22 of copper. A coating of shellac 23 may be applied to the copper to mask the copper against electrolytic deposit when subjected to an electrolytic bath for the production of foraminous sheet.

The structure thus far described is illustrated in Fig. 4, where the numeral 24 indicates depressions, and the numeral 25 indicates the peripheral ledges on the walls of the depressions.

The depressions 24 may now be filled with passive material 27 consisting, for example, of Bakelite, and the entire surface rubbed to as perfect a plane as possible, leaving lands 26 of exposed metal defining the pattern of the foraminous sheet to be produced and with the passive material 27. This composite plate may then be employed as a cathode in an electrolytic bath for the deposition of foraminous sheet. It is, of course, necessary prior to the latter step that a stripping film be applied to the lands 26, of such a character that while the lands will receive a deposit, the deposit will not adhere tenaciously enough to prevent ready stripping.

As regards the passive material 27, it will be noted that the mass is firmly locked in position

by the ledges 25, and for this reason the matrix will withstand continued and repeated use.

In producing the matrix, it is desirable to provide for a selvage edge along the borders thereof, as it is usual to produce foraminous sheet in which openings do not extend to the extreme limit of the sheet. It is desirable, therefore, to provide on the upper peripheral face a cutaway portion 28. This cutaway portion is coated with the wax and graphite mixture 14 and as a result the layer 15 has a portion 29 which conforms to the shape of the cutaway portion. In the finished matrix this cutaway portion is duplicated in the layer 21, as indicated by the reference numeral 30 and is filled with insulating material as 31 indicated by the reference numeral 31 in Fig. 4.

I have described above certain embodiments of my invention and a preferred process with certain modifications thereof, but I wish it to be understood that these are illustrative and not limitative of my invention and that I reserve the right to make various changes in form, construction, and arrangement of parts and also to make various changes in process of manufacture falling within the spirit and scope of my invention, as set forth in the claims.

I claim:

1. In the method of making a matrix, the steps which comprise forming a plate of metal with a plurality of projections on one face thereof, coating the surface of the plate of metal around the base of the projections with a non-conductive material, electro-depositing metal on the surface of the projections to an extent to overlie the non-conductive material, removing the non-conductive material and then depositing a layer of metal on the surface of the plate having the projections thereon, and then dissolving the plate of metal.

2. The improved method of making a matrix, which comprises forming a plate of metal with a plurality of projections on one face thereof, coating the surface of the plate around the base of the projections with a non-conductive material, electro-depositing metal on the surface of the projections to overlie the non-conductive material, removing the non-conductive material from the plate, depositing a layer of metal on the surface of the plate of metal and on the projections, dissolving the plate of metal, and then filling the depressions in the layer of metal with non-conductive material.

3. The improved method of making a matrix, which comprises forming a plate of metal with a plurality of projections on one face thereof, coating the surface of said plate of metal around the base of the projections with a soluble non-conductive material, electro-depositing metal on the surface of the projections to form a peripheral shoulder around each projection, removing the soluble non-conductive material, depositing a layer of metal on the surface of the plate having the projections thereon, removing the plate of metal, and filling the depressions in the layer of metal with insulating material.

4. The improved method of making a matrix, which comprises forming a plate of metal with a plurality of projections on one face thereof, coating the surface of said plate around the base of the projections with a soluble non-conductive material, electro-depositing metal on the exposed surface of the projections to accentuate the height of the projections and form a peripheral groove around each projection, dissolving the soluble non-conductive material, depositing a

layer of metal on the surface of the plate of metal having the projections thereon to produce a matrix base, dissolving the plate of metal so that only the layer of metal remains, and filling the 5 depressions in the layer of metal with insulating material.

5. In the improved method of making a matrix having one face thereof provided with a plurality of indentations arranged in any desired 10 pattern and with each indentation isolated from every other indentation, the steps which comprise making a master plate by electro-depositing metal and in which the indentations which are to appear in the matrix assume the form of 15 projections, coating the face of the master plate around the base of the projections with a non-conductive material, electro-depositing metal on the face of the master plate and on the projections to accentuate the height of the projections 20 and form circumferential grooves around each projection, removing the non-conductive material, depositing a layer of metal on the master plate, and then removing the master plate.

6. The improved method of making a matrix, 25 which comprises forming a plate of metal with a plurality of projections thereon, coating the surface of the plate around the base of the projections with a soluble non-conductive material,

electro-depositing metal on the exposed surface of the projections on the plate of metal to accentuate the height of the projections and form a peripheral groove around each projection, dissolving the soluble non-conductive material, depositing a layer of metal on the surface of the plate of metal having the projections thereon to produce a matrix, dissolving the plate of metal so that only the matrix remains, and filling the 5 depressions in the matrix with insulating material. 10

7. The improved method of making a matrix for the electrodeposition of foraminous sheet, which comprises forming a plate of metal with a plurality of protuberances on one face thereof, 15 coating the said face around the bases of the protuberances with electrically non-conductive material, electrodepositing metal on the surface of the protuberances to form a peripheral shoulder around each protuberance, removing the electrically non-conductive material, electrodepositing a layer of metal on that surface of the plate on which the protuberances are located, removing the first-mentioned plate with its protuberances, and filling the depressions in the last-mentioned plate with electrically non-conductive 20 material. 25

EDWARD O. NORRIS.